

# UNITED STATES PATENT OFFICE.

FRANK K. CAMERON AND JOHN A. CULLEN, OF SALT LAKE CITY, UTAH, AND REED W. HYDE, OF NEW YORK, N. Y., ASSIGNEES TO AMERICAN SMELTING & REFINING COMPANY, OF SALT LAKE CITY, UTAH, A CORPORATION OF NEW JERSEY.

## METHOD OF TREATING SULFID ORES.

1,261,694.

Specification of Letters Patent.

Patented Apr. 2, 1918.

No Drawing.

Application filed June 18, 1917. Serial No. 175,529.

To all whom it may concern:

Be it known that we, (1) FRANK K. CAMERON, (2) JOHN A. CULLEN, and (3) REED W. HYDE, citizens of the United States, 5 residing at (1) Salt Lake City, (2) Salt Lake City, and (3) New York city, in the counties of (1) Salt Lake, (2) Salt Lake, and (3) New York, and States of (1) Utah, (2) Utah, and (3) New York, have invented cer- 10 tain new and useful Improvements in Methods of Treating Sulfid Ores, of which the following is a specification.

This invention is a method of treating sulfid ores for the recovery therefrom of the 15 metal values and elemental sulfur. The method will be described in its application to complex sulfids carrying one or more sulfids of zinc, lead, copper and iron, together with some silver, gold and manganese, with 20 other components and gangue minerals.

We have discovered that in presence of strong sulfuric acid and at high temperatures, these sulfid ores undergo decomposition, yielding elemental sulfur which distils 25 from the mass, and the sulfates of the metals which remain as a residue. The reaction probably takes place in stages, and is not achieved or realized in practice in a complete form; but it may be summarized in the 30 following ideal equation which is more or less imperfectly approximated, namely:—



35 A more or less close approximation to this reaction is obtained when the ore, mixed with sulfuric acid having a concentration of 50° Baumé or higher, is raised quickly to a temperature of about 200° C., more or less.

40 The sulfid ore may be simply mixed with the sulfuric acid in about the proportions above described and the mixture quickly heated to the required temperature. We prefer however, in order to secure more 45 nearly uniform temperature conditions and a better approximation to the ideal reaction, to heat the sulfuric acid first nearly to its boiling point, and then to add the ore.

The reaction is carried out in a still or vessel which may be of cast iron, air or other extraneous sources of oxygen being excluded during the operation.

Under such conditions some hydrogen sulfid is first generated, followed by the evo-

lution of sulfur dioxid, and presently if the 55 temperature be sufficiently maintained by a copious evolution of elemental sulfur, mixed with water-vapor, sulfur dioxid and sulfur trioxid, or with vapors of sulfuric acid. The sulfur is easily condensed and recovered 60 and may be marketed as such, while the oxids of sulfur can readily be collected, re-converted into sulfuric acid, or find other economical uses.

When the reaction is complete, as evi- 65 denced by the cessation of evolution of sulfur or oxids of sulfur, the mass is allowed to cool somewhat and is lixiviated with wa- 70 ter. We obtain thereby an aqueous solution containing practically all of the zinc, to- 75 gether with more or less ferrous iron, copper, aluminum, silver, etc. By well known and commonly practised methods all bases other than zinc are readily removed, leav- 80 ing a technically pure solution which may be 85 used for the production of zinc sulfate, or of the chlorid or other salts of zinc, or which may be electrolyzed for the production of the metal. The precipitated iron, silver, etc., from the zinc sulfate solution may profitably 80 be added to the extracted residue, consisting mainly of lead sulfate but containing also gold, silver, silica, manganese, etc., and the mixture sent to the lead smelter.

While we prefer to heat the acid to a high 85 temperature before adding the ore, our invention is not limited to this or other specific manipulation. The more quickly the mixture is brought to the requisite tempera- 90 ture, the more closely the reaction will approach the ideal equation as above expressed. We consider therefore that any method whereby such rapid heating may be accomplished is equivalent to that described herein. The application of the principle of 95 Le Chatelier indicates that an increased yield of sulfur may be expected by carrying out the reaction under increased pressure.

We claim:—

1. The method of recovering elemental 100 sulfur and metal values from sulfid ores, which consists in reacting thereon with strong sulfuric acid at a temperature approximating the boiling-point of the acid, distilling off sulfur, and recovering the 105 metal values from the residue.

2. The method of recovering elemental sulfur and metal values from sulfid ores,

which consists in quickly heating sulfid ore and strong sulfuric acid to a reacting temperature approximating the boiling-point of the acid, distilling off sulfur, and recovering the metal values from the residue.

3. The method of recovering elemental sulfur and metal values from sulfid ores, which consists in heating sulfuric acid having a concentration of at least 50° Baume

approximately to its boiling-point, adding <sup>10</sup> thereto a sulfid ore, distilling off sulfur, and recovering the metal values from the residue.

In testimony whereof, we affix our signatures.

FRANK K. CAMERON.  
JOHN A. CULLEN.  
REED W. HYDE.